

## UNITED STATES PATENT OFFICE

WILLIAM J. MERTEN, OF PITTSBURGH, PENNSYLVANIA, ASSIGNOR TO WESTINGHOUSE ELECTRIC &amp; MANUFACTURING COMPANY, A CORPORATION OF PENNSYLVANIA

## PROCESS FOR PURIFYING METALS AND THE PRODUCT PRODUCED THEREBY

No Drawing.

Application filed June 4, 1927. Serial No. 196,635.

My invention relates to alloys and specifically to non-ferrous alloys in which lead is one of the constituents and to methods of making the same.

5 It is among the objects of my invention to provide a non-ferrous alloy in which a comparatively soft constituent is widely and uniformly disseminated in a matrix of harder and stronger metal.

10 Another object of my invention is to provide a bearing metal of improved characteristic which possesses better wearing properties than alloys of similar chemical composition.

15 Alloys containing lead 10% to 28%, tin 2% to 10%, and the remainder copper and minor impurities have hitherto been made. Such bronze alloys have been used extensively for bearings as the alloy structure consists of lead or a soft lead alloy existing in

20 and dispersed in a matrix of harder metal or alloy consisting mainly of copper. The soft selectively segregated particles of lead in the harder matrix provides the kind of

25 surface in bearings which will compensate in some measure for oil lubrication when the film of lubricating oil becomes temporarily broken, provided the soft metal or lubricating constituent is more or less uniformly distributed throughout the matrix.

30 Heretofore, bearings which were made of such alloys have not been uniformly satisfactory because of the lack of uniform distribution of the soft lubricating metal in the harder matrix and because of segregation of the lead. The segregation of the lead results in an excess of lead in certain portions of the structure and too little or no lead in other portions.

35 I have discovered that when the alloy is treated in the molten state with calcium carbide ( $CaC_2$ ), the lead is caused to disseminate and to be mechanically dispersed into extremely small spheroidal bodies throughout the matrix, and that segregation of the lead is prevented thereby. The bodies of lead appear to be slightly harder, they are more tenacious and less friable than metallic lead and a tight efficient bonding with

40 the cuprous metal crystals exists.

When the melted alloy is treated in accordance with my process, there is an evolution of gas comprising oxides of carbon which are derived from the combination of the carbon in the calcium carbide with the 55 oxides in the alloy. A dross or slag-like material that contains silicates, sulphates and other impurities is formed and rises to the surface of the melt. It would be expected that the elimination of the hard compounds 60 comprising oxides and other non-metallic compounds in the alloy would soften it, but on the contrary, the alloy is noticeably harder than untreated alloys of like composition. It is believed that the improved properties 65 of the alloy is due to the presence of calcium as a calcium-lead compound as well as to the existence of the lead in a new physical character with respect to the matrix.

The hardened alloy is particularly useful 70 for bearings since it is less apt to be distorted when it is subjected to a heavy pressure, therefore, a bearing made of the alloy will retain its intended shape and proportions 75 for a long time in service. The lead operates to impart the property of lubrication to the alloy as it is uniformly distributed and dispersed throughout the structure. Consequently, the alloy is a material that is 80 resistant to distortion and has a small amount 85 of uniformly distributed softer metal or lubricant in it. These characteristics are believed to account for the improved wearing qualities of bearings that are made of my new alloy.

I provide an alloy consisting of lead 10% to 28%, tin 2% to 10% and copper and impurities 88% to 62%. The alloy is made by melting the constituents together in the desired proportions. When the alloy is melted, or if preferred, during the melting of the alloy, I add calcium-carbide in the proportion of about one pound of carbide to fifty pounds of the alloy. The calcium-carbide reacts with the impurities, such as oxides and produces gases and slag-like materials that separate from the metal. The calcium compounds of slag-like material are lighter than the metallic compounds of lead 90 95 100

and they can be removed from the surface of the melt with the dross.

In addition to its cleaning or scavenging action, calcium-carbide appears to harden the lead and to cause a spheroidal dispersion of the lead throughout the alloy. It appears from microscopic examination that there has been a physical change in the lead constituent and that it is disseminated in a matrix of the stronger and harder metal in fine well distinguished globules which occur as definite distinct spheroidal aggregates of metallic crystals disposed among the copper-metal crystals and not as an accumulation or segregation of lead of planiform or indefinite form and amount at the crystal boundaries, such as the segregation occurring in untreated alloys of like chemical analysis.

Although I have described a specific alloy and a specific modification of my process, I do not wish to be limited thereto, as a similar dispersion of the soft insoluble constituent of other non-ferrous alloys may be produced by utilizing my invention. Other modifications of my invention will suggest themselves to those skilled in the art without departing from the spirit of my invention as defined by the appended claims.

I claim as my invention:

1. In the process of preparing alloys comprising at least 62% copper, a small percentage of tin and the remainder lead, the step which comprises adding calcium carbide to the alloy when it is in at least a partially molten state for the purpose of causing a dispersion of the lead throughout the copper-tin matrix and preventing its segregation during the subsequent cooling of the alloy.

2. In the process of preparing alloys comprising at least 62% copper, 2% to 10% tin and the remainder lead, the steps which comprise melting the constituents of the alloy together, adding calcium carbide to the melted alloy and then cooling the alloy.

3. In the process of preparing alloys comprising from 62% to 88% copper, 2% to 10% tin and the remainder lead and minor impurities, the steps which comprises melting the ingredients together, adding calcium carbide to the molten alloy, removing the impurities from the surface of the metal and then cooling the alloy.

4. In the process of preparing alloys comprising 10% to 28% lead, 2% to 10% tin and 62% to 88% copper and minor impurities, the steps which comprise melting the ingredients together, adding calcium carbide to the molten alloy and then permitting the alloy to cool.

In testimony whereof, I have hereunto subscribed my name this 27th day of May, 1927.